

Patented June 11, 1925

1,716,420

UNITED STATES PATENT OFFICE.

STEWART J. CARROLL, OF ROCHESTER, NEW YORK, ASSIGNOR TO EASTMAN KODAK COMPANY, OF ROCHESTER, NEW YORK, A CORPORATION OF NEW YORK.

CELLULOSE-ETHER FILM AND COMPOSITION FOR MAKING THE SAME.

No Drawing.

Application filed August 9, 1926. Serial No. 128,337.

This invention relates to compositions of matter in which cellulose ethers, such as water-insoluble ethyl cellulose, are combined or mixed with other substances which impart not only low inflammability, but likewise give compositions the other properties of which are also highly advantageous in the plastic and analogous arts, such, for instance, as the film or varnish arts.

10 One object of the invention is to provide cellulose ether films having not only all of the ordinary desirable qualities of films for photographic purposes, but also having unusually low inflammability and extremely 15 high resistance to deterioration by heating. Another object of the invention is to provide permanently transparent, strong, flexible sheets or films of desired thinness, which are substantially waterproof, are unaffected 20 by ordinary photographic fluids, are substantially colorless, are substantially without harmful action upon light-sensitive photographic coatings, are of low inflammability and highly resistant to prolonged heat. An- 25 other object of the invention is to provide compositions capable of easy manipulation in film making, varnish making, or allied plastic arts. Another object is to provide compositions which will not injure or be in- 30 jured by the substances or surfaces with which they are associated during manufacture, storage or use. Other objects will hereinafter appear.

In U. S. Patent No. 1,188,376, Lilienfeld, 35 June 20th, 1916, there are disclosed a series of alkyl ethers of cellulose. Certain of these are particularly insoluble in water, and the present invention finds its chief value in connection with ethers having this property, 40 such as water-insoluble ethyl cellulose, films of which have small shrinkage characteristics, after treatment in photographic baths. In U. S. Patent No. 1,583,709, Webb, May 4th, 1926, there are disclosed films of such 45 cellulose ethers in which the ordinary desirable qualities of photographic film base are combined with resistance to prolonged heating, this result being brought about by maintaining an alkalinity in excess of  $\text{Ph}_7$ . It is 50 desirable that such films, especially motion picture films, be capable of withstanding heating without becoming brittle. Whether or not films will possess this property can be foretold with practical accuracy by testing samples, say by heating them for weeks 55

and even months at a continuous temperature of  $65^{\circ}$  C. Films which remain usefully flexible after such a severe test are capable of withstanding the conditions met with in use.

I have found that these qualities of the films may be maintained and yet the inflammability greatly lowered by incorporating in such films and in the compositions out of which they are made, one or more of the brom-nucleo substitution products of benzol and its homologues, especially those which are liquid at ordinary temperatures and have saturated side chains, such, for example, as mono, di, tri, or other poly brom benzols, toluenes, xylenes, mesitylenes, ethylbenzenes, cumenes and cymenes. Where ortho, meta or para isomers exist, they are all usable. On account of their relative cheapness and simplicity of manufacture, I prefer mono-brombenzol, parabromtoluene, and ortho-bromtoluene. All of these substances, when mixed into the film-making compositions, should be free from free bromine and free hydrobromic acid. Otherwise they will cause sufficient discoloration to make the film undesirable for photographic purposes, will cause deterioration of any photographic emulsions placed upon the film, and will destroy the alkalinity upon which the resistance of the film to prolonged heating depends. If the brominated compounds are initially purified from free bromine and free hydrobromic acid and are incorporated in films having an alkalinity greater than  $\text{Ph}_7$ , there is no acidity in the film-making solution, nor in the film, nor does this condition develop during the normal storage of the solution or during the normal useful life of the film.

I shall now give one example of my invention by way of illustration, but it will be understood that the invention is not limited to these details, except as indicated in the appended claims. 100 parts by weight of water-insoluble ethyl cellulose containing sufficient alkali, say by undergoing the treatment given in lines 78 to 92 of page 1 in the above cited Webb patent, are dissolved along with 5 to 50 (say 10 parts) of mono-brombenzol in 300 to 500 parts of a volatile common solvent. The latter may usefully comprise a mixture of methyl acetate and methyl alcohol, the weight of the methyl acetate being approximately nine times the 105 110

weight of the methyl alcohol. Of course, the ingredients of the solvent are of sufficient purity to avoid acidifying the composition. This composition is suitable for 5 spreading upon a film-forming surface in a coating, from which the volatile solvent evaporates sufficiently to leave a transparent, flexible sheet, which is stripped off and otherwise treated in a manner well known 10 to those skilled in this art. In place of the monobrombenzol, an equal number of parts by weight can be substituted of any one of the brominated bodies mentioned hereinabove, or mixtures of them. By reason of 15 the fact that these brominated products are of the nucleo type, having the bromine atoms directly bonded to the ring of carbon atoms, they are particularly stable.

The ingredients in the film-forming composition are thoroughly mixed and may be 20 filtered if desired. When more flowable solutions are desired, or when the compositions are to be employed as lacquers, the volatile solvent may be increased until the 25 desired viscosity is obtained, or volatile liquids, such as benzol, alcohol, and the like may be added to the thinner. Along with the ingredients mentioned above, I may add one or more supplementary organic bodies 30 of only slight volatility which enhance the flexibility of the compositions and regulate the preparation of film therefrom; but such bodies are not essential. Examples of them are amyl or butyl acetate, the various amyl 35 alcohols, the various butyl alcohols, and mixtures of them. Of course, these ingredients are also sufficiently pure to be non-acid.

Films prepared from the hereinabove described compositions are flexible, smooth, 40 transparent, strong, substantially colorless, substantially waterproof, are unaffected by ordinary photographic baths, and in addition, combine unexpectedly low inflammability with high resistance against brittleness upon prolonged heating at 65° C., or 45 equivalent conditions in actual use. The amount of alkali in the film is, of course, insufficient to impair their transparency.

Having thus described my invention, what 50 I claim as new and desire to secure by Letters Patent is:

1. A flowable composition comprising a water-insoluble cellulose ether, a brom-nucleo substitution product of benzol and its 55 homologues, which product is substantially free from uncombined bromine and hydrobromic acid, and a solvent common to said ingredients, said composition being stabili-

lized by the presence therein of inorganic alkali which creates an alkalinity in the 60 composition in excess of Ph., the proportions being such that a product formed therefrom will have the properties of high transparencies, freedom from accidental color, inertness toward photographic emulsions and 65 high resistance to heating.

2. A composition of matter comprising substantially the following: 100 parts by weight of water insoluble ethyl cellulose, 10 parts of monobrombenzol substantially free 70 from uncombined bromine and hydrobromic acid, and more than 300 parts of a volatile common solvent, said composition comprising sufficient inorganic alkali to give it an alkalinity in excess of Ph. 75

3. A flowable composition comprising 100 parts by weight of water-insoluble ethyl cellulose, 5 to 50 parts of monobrombenzol substantially free from uncombined bromine and hydrobromic acid, and more than 300 80 parts of a volatile common solvent, said composition comprising sufficient inorganic alkali to give it an alkalinity in excess of Ph., the proportions being such that a product formed therefrom will have the properties of high transparencies, freedom from 85 accidental color, inertness toward photographic emulsions and high resistance to heating.

4. As an article of manufacture, a film 90 comprising colloidized water-insoluble cellulose ether and a brom-nucleo substitution product of benzol and its homologues, said product being substantially free from uncombined bromine and hydrobromic acid, 95 said film having distributed therein sufficient inorganic alkali to give the film an alkalinity in excess of Ph., the proportions of the ingredients being such that the film is flexible, transparent and inert to photographic emulsions. 100

5. As an article of manufacture a film comprising colloidized water-insoluble ethyl cellulose and monobrombenzol free from uncombined bromine and hydrobromic acid, said film having uniformly distributed therein sufficient inorganic alkali to give the film an alkalinity in excess of Ph., the amount of alkali being insufficient to impair 110 the transparency of the film, the proportions of the ingredients being such that the film is flexible, transparent and inert to photographic emulsions. 105

Signed at Rochester, New York, this 29th day of July, 1926.

STEWART J. CARROLL.